

## UNITED STATES PATENT OFFICE.

JAMES DAVID LUMSDEN, DECEASED, LATE OF ALMONDBANK, SCOTLAND, BY SUSAN A. R. F. LUMSDEN, OF ALMONDBANK, ROBERT W. R. MACKENZIE, OF EARLSSHALL, JOHN G. MILLER, OF PERTH, ROBERT O. LUMSDEN, OF ALMONDBANK, AND ALEXANDER P. MELVILLE, OF EDINBURGH, SCOTLAND, EXECUTORS, AND ROBERT W. R. MACKENZIE, OF EARLSSHALL, ERNEST H. ROBINSON, OF PERTH, AND MORRIS FORT, OF ALMONDBANK, SCOTLAND.

SCOURING AND BLEACHING OF YARNS AND FABRICS COMPOSED OF VEGETABLE FIBERS  
CONTAINING DYED-EFFECT THREADS OR FIBERS.

No Drawing.

Application filed March 23, 1921. Serial No. 454,933.

(GRANTED UNDER THE PROVISIONS OF THE ACT OF MARCH 3, 1921, 41 STAT. L., 1313.)

To all whom it may concern:

Be it known that we, SUSAN ANN RANKINE FORTUNE LUMSDEN, widow of JAMES DAVID LUMSDEN, deceased, a resident of Almondbank, Perthshire, Scotland, ROBERT WALKER RANNIE MACKENZIE, a resident of Earlshall, Fife, Scotland, JOHN GARDNER MILLER, a resident of Perth, Perthshire, Scotland, ROBERT OSWALD LUMSDEN, a resident of Almondbank, Perthshire, Scotland, and ALEXANDER PATRICK MELVILLE, a resident of Edinburgh, Scotland, all subjects of the King of Great Britain, Ireland, and the Isle of Man, are executors of the estate of JAMES DAVID LUMSDEN, formerly a resident of Huntingtowerfield, Almondbank, Perthshire, Scotland, but now deceased, and that we, ROBERT WALKER RANNIE MACKENZIE, a resident of Earlshall, Fife, Scotland, ERNEST HOWARD ROBINSON, a resident of Stornoway, Perth, Scotland, and MORRIS FORT, a resident of Almondbank, Perthshire, Scotland, all British subjects, jointly with the late JAMES DAVID LUMSDEN aforesaid have invented new and useful improvements in and relating to the scouring and bleaching of yarns and fabrics composed of vegetable fibers containing dyed-effect threads or fibers, (for which we have filed an application in Great Britain March 20, 1920, Patent No. 165,198), of which the following is a specification.

This invention has reference to our improved process of scouring and bleaching cotton and linen yarns and fabrics containing dyed effect fibers or threads, whereby the well-known difficulty of avoiding bleeding and staining during boiling or scouring with alkaline solutions is largely or entirely overcome. By application of our invention the dyed colours are also better preserved, the fabrics yield a superior finish and appearance, and in many cases a much better white can be obtained than by any known scouring and bleaching operations hitherto applied to this class of material.

We carry out our invention by making preliminary tests as to the nature and behaviour

of the dyed portions of yarns and fabrics when extracted with volatile organic solvents such as benzol, naphtha, benzine. In only very few cases among the bleaching colours in present use, with the exception of a few indigoid vat dyes, will solvent extraction, hot or cold, seriously affect the colour of dyed fibers or threads to cause staining or excessive bleeding. Other solvents than these also may be used, for example alcohol and chlorinated hydrocarbons, but these latter are more likely to affect the dyed shades than the examples of hydrocarbons solvents given. We then proceed to carry out extraction of the goods in bulk with a suitable volatile organic solvent whereby are eliminated from the fabrics substantial amounts of impurities, chiefly oil, fat and wax and allied and associated matter for the removal of which alkaline scouring or boiling has hitherto been applied.

The extraction with solvents may be carried out by use of any known method and apparatus and the solvent employed recovered as well as the extracted oily, fatty and waxy matter by steaming, distillation and other known means of recovery. Thereafter a much shorter or milder scouring with alkaline solutions than is usually required, or is otherwise permissible, may be given to the goods, as for example, boiling without pressure where otherwise pressure is required, or saturation with hot weak alkaline solutions by running through a machine or by passing hot alkaline solutions through the goods instead of boiling with alkali, or sodium carbonate may replace the use of caustic soda, or caustic soda the use of lime, or in the case of some cotton fabrics alkaline treatments may be omitted altogether and yet satisfactory whites may be obtained by chemicing and scouring after the solvent extraction we propose.

It has been proposed previously to bleach cotton and linen goods white after solvent extraction and subsequent boiling without reference to the preservation of dyed fibers liable to bleed on boiling with alkalis, and

we make no claim herein to the treatment of any class of goods other than these containing dyed effect threads or fibers, our invention being solely concerned with the 5 preservation of these from bleeding and staining during scouring and bleaching treatment by a preliminary solvent treatment which allows of eliminating or reducing the severity of alkaline scouring in 10 a manner favourable to the preservation of dyed colours in the goods undergoing treatment.

It has been proposed and patented previously by us to extract with solvents linen 15 and cotton goods, including goods also containing dyed threads in order to ensure good beetling properties. It is now claimed as our invention to extract such goods which require to be bleached but may or may not 20 require to be beetled.

Our invention is also applicable to the scouring and bleaching of yarns and fabrics consisting entirely of dyed fibers in which the dyed shades are required to withstand 25 the subsequent scouring and bleaching of the fibers upon which they are dyed.

What we claim is:—

1. The process of scouring linen and cotton yarns and fabrics containing dyed 30 threads or fibers, which comprises treating said yarns and fabrics with a volatile organic solvent to remove impurities, and

thereafter subjecting the said articles to a comparatively mild scouring operation with alkaline solution.

2. The process of scouring linen and cotton yarns and fabrics containing dyed threads or fibers, which comprises treating said yarns and fabrics with a volatile organic solvent to remove impurities, and subjecting the said articles to a comparatively mild scouring operation with alkaline solution, in conjunction with subsequent bleaching operations, substantially as described.

S. A. R. F. LUMSDEN.

R. W. R. MACKENZIE.

J. G. MILLER.

R. O. LUMSDEN.

ALEX. P. MELVILLE.

*Executors of James David Lumsden, deceased.*

R. W. R. MACKENZIE,

ERNEST H. ROBINSON.

MORRIS FORT.

Witnesses to the signatures of S. A. R. F. Lumsden, R. W. R. Mackenzie, J. G. Miller, R. O. Lumsden, Ernest H. Robinson, and Morris Fort:

D. A. COATES,

D. A. R. CUTHBERT.

Witnesses to the signature of Alex. P. Melville:

ALASTAIR H. CREVAR,

JOHN H. M. SOMERVILLE.